



US010734157B2

(12) **United States Patent**  
**Park**

(10) **Patent No.:** **US 10,734,157 B2**  
(b5) **Date of Patent:** **Aug. 4, 2020**

(54) **INDUCTOR**

(71) **Applicant:** **SAMSUNG ELECTRO-MECHANICS CO., LTD.**  
Suwon-si, Gyeonggi-do (KR)

(72) **Inventor:** **Jong Ik Park**, Suwon-si (KR)

(73) **Assignee:** **SAMSUNG ELECTRO-MECHANICS CO., LTD.**  
Suwon-si, Gyeonggi-Do (KR)

(\*) **Notice:** Subject to any disclaimer, the term of this patent is extended or adjusted under 35 U.S.C. 154(b) by 129 days.

(21) **Appl. No.:** **15/002,132**

(22) **Filed:** **Jan. 20, 2016**

(65) **Prior Publication Data**

US 2016/0322154 A1 Nov. 3, 2016

(30) **Foreign Application Priority Data**

Apr. 29, 2015 (KR) ..... 10-2015-0060289

(51) **Int. Cl.**

**H01F 5/00** (2006.01)  
**H01F 17/00** (2006.01)  
**H01F 27/29** (2006.01)  
**H01F 17/04** (2006.01)

(52) **U.S. Cl.**

CPC ..... **H01F 27/292** (2013.01); **H01F 17/0013** (2013.01); **H01F 17/04** (2013.01); **H01F 2017/048** (2013.01)

(58) **Field of Classification Search**

CPC .... H01F 17/0013; H01F 22/292; H01F 5/003;  
H01L 2924/30107

USPC ..... 336/200; 257/531; 29/6021  
See application file for complete search history.

## (56)

**References Cited**

## U.S. PATENT DOCUMENTS

3,590,480 A \* 7/1971 Johnson, Jr. ..... H01F 19/08  
174/528  
4,217,689 A \* 8/1980 Fujii ..... H01L 21/3043  
125/13.01  
4,610,079 A \* 9/1986 Abe ..... H01L 21/3043  
148/DIG. 28  
4,814,296 A \* 3/1989 Jedlicka ..... B27G 19/10  
148/DIG. 28  
4,853,815 A \* 8/1989 Diepers ..... G11B 5/1278  
360/125.06  
4,860,433 A \* 8/1989 Miura ..... H01F 27/292  
29/605

(Continued)

## FOREIGN PATENT DOCUMENTS

JP 2001266431 A \* 9/2001  
JP 2004-342814 A 12/2004

(Continued)

## OTHER PUBLICATIONS

Office Action issued in corresponding Korean Patent Application No. 10-2015-0060289 dated Oct. 30, 2019, with English translation.

*Primary Examiner* — Elvin G Enad

*Assistant Examiner* — Joselito Baisa

(74) **Attorney, Agent, or Firm:** Morgan, Lewis & Bockius LLP

(57) **ABSTRACT**

An inductor includes a magnetic body including a magnetic substance; a substrate disposed within the magnetic body; and an internal electrode disposed on at least one of an upper surface and a lower surface of the substrate. The substrate is disposed on an inclined with respect to at least one surface of the magnetic body.

**16 Claims, 5 Drawing Sheets**



| (56)                  | References Cited      |              |            |                          |                        |              |  |  |
|-----------------------|-----------------------|--------------|------------|--------------------------|------------------------|--------------|--|--|
| U.S. PATENT DOCUMENTS |                       |              |            |                          |                        |              |  |  |
| 5,022,141 A *         | 6/1991 Nagata .....   | G11B 5/3163  | 29/603.24  | 2006/0214759 A1*         | 9/2006 Kawarai .....   | H01F 17/0006 |  |  |
| 5,157,576 A *         | 10/1992 Takaya .....  | H01F 17/0006 | 257/531    | 2007/0146109 A1          | 6/2007 Nogi .....      | 336/200      |  |  |
| 5,189,949 A *         | 3/1993 Apa .....      | A47J 31/4485 | 99/323.3   | 2007/0182519 A1*         | 8/2007 Tsuzuki .....   | H01F 17/0006 |  |  |
| 5,245,493 A *         | 9/1993 Kawabe .....   | G11B 5/012   | 360/119.05 | 2008/0055859 A1*         | 3/2008 Furukawa .....  | H01C 1/148   |  |  |
| 5,805,391 A *         | 9/1998 Chang .....    | G11B 5/23    | 360/122    | 2009/0067110 A1*         | 3/2009 Beyer .....     | 361/704      |  |  |
| 6,055,976 A *         | 5/2000 Davies .....   | B23D 61/10   | 125/13.01  | 2010/0271163 A1*         | 10/2010 Nakamura ..... | H01H 9/0072  |  |  |
| 6,296,776 B1*         | 10/2001 Sasaki .....  | G11B 5/3116  | 216/22     | 2011/0069363 A1*         | 3/2011 Chikaoka .....  | 361/191      |  |  |
| 6,504,463 B1*         | 1/2003 Kato .....     | H01F 27/292  | 336/83     | 2011/0158276 A1*         | 6/2011 Takagi .....    | B32B 18/00   |  |  |
| 7,190,553 B2*         | 3/2007 Morita .....   | G11B 5/3116  | 360/125.39 | 2012/0012632 A1*         | 1/2012 Tominaga .....  | 336/200      |  |  |
| 7,304,557 B2*         | 12/2007 Tsuzuki ..... | H01F 17/0006 | 336/200    | 2012/0032307 A1*         | 2/2012 Tomita .....    | B28D 1/24    |  |  |
| 7,446,638 B2*         | 11/2008 Nogi .....    | H01F 3/14    | 336/200    | 2013/0249662 A1*         | 9/2013 Tonoyama .....  | 225/2        |  |  |
| 7,989,320 B2*         | 8/2011 Boyle .....    | H01L 21/6836 | 257/782    | 2014/0167897 A1          | 6/2014 Choi et al.     | 257/618      |  |  |
| 8,975,997 B2*         | 3/2015 Tonoyama ..... | H01F 27/255  | 336/200    | 2014/0176283 A1*         | 6/2014 Yang .....      | H01F 41/046  |  |  |
| 9,966,498 B2*         | 5/2018 Tsai .....     | H01L 33/46   | 336/200    | 2016/0042997 A1*         | 2/2016 Takahashi ..... | 336/200      |  |  |
| 2002/0158547 A1*      | 10/2002 Wood .....    | B81B 3/0054  | 310/307    |                          |                        | 438/464      |  |  |
| 2003/0025085 A1*      | 2/2003 Nakano .....   | B82Y 10/00   | 250/396 ML | FOREIGN PATENT DOCUMENTS |                        |              |  |  |
| 2006/0152321 A1*      | 7/2006 Jung .....     | H01F 17/0006 | 336/200    | JP                       | 2007-157983 A          | 6/2007       |  |  |
|                       |                       |              |            | JP                       | 2009-49046 A           | 3/2009       |  |  |
|                       |                       |              |            | KR                       | 10-2006-0061709 A      | 6/2006       |  |  |
|                       |                       |              |            | KR                       | 10-2006-0081493 A      | 7/2006       |  |  |
|                       |                       |              |            | KR                       | 10-2014-0077346 A      | 6/2014       |  |  |

\* cited by examiner



FIG. 1



FIG. 2

200

FIG. 3



FIG. 4



FIG. 5

# 1 INDUCTOR

## CROSS-REFERENCE TO RELATED APPLICATION

This application claims the benefit of priority to Korean Patent Application No. 10-2015-0060289, filed on Apr. 29, 2015 with the Korean Intellectual Property Office, the entirety of which is incorporated herein by reference.

## TECHNICAL FIELD

The present inventive concept relates to an inductor.

## BACKGROUND

An inductor, together with a resistor and a capacitor, is a key passive element constituting an electronic circuit. Inductors are used in components to cancel noise or to form an LC resonance circuit. Inductors may be classified as winding type inductors, laminated type inductors, thin film type inductors, and the like, according to the structure thereof.

A winding type inductor may be formed by winding a coil around a ferrite core. A winding type inductor may have stray capacitance generated between coil portions, and accordingly, when the number of turns of a coil is increased to obtain high capacity inductance, degradation of high frequency characteristics may occur.

A laminated type inductor may be formed by laminating a plurality of ceramic sheets. In a laminated type inductor, coil-like metal patterns are formed on respective ceramic sheets, and the coil-like metal patterns may be sequentially connected to one another by a plurality of conductive vias provided in the ceramic sheets. Laminated type inductors are appropriate for mass-production, and have excellent high frequency characteristics compared to winding type inductors.

However, in a laminated type inductor, metal patterns are formed of a material having a low saturation magnetization value. When a laminated type inductor is manufactured to have a small size, the number of laminations of the metal patterns is limited, and this may lead to a degradation in DC superposition characteristics, thereby resulting in a failure to obtain a sufficient current.

A thin film type inductor may use a material having a high saturation magnetization value, and even when a thin film type inductor is manufactured to have a small size, an internal circuit pattern thereof may be easily formed in comparison to a laminated type inductor. Thus, research has been actively undertaken into thin film type inductors.

When a thin film type inductor is manufactured on a large scale, a line width or thickness of a coil may be increased, thereby eliminating degradation in product characteristics due to an increase in series resistance.

However, when a thin film type inductor is manufactured to have a small size, an increase in the line width or thickness of a coil is limited. Thus, delamination, cracks, and the like may occur between internal electrodes formed within the inductor and a substrate, and between magnetic substances of an inductor body during a chip-cutting process.

## SUMMARY

An aspect of the present inventive concept provides an inductor having high capacity characteristics and allowing

# 2

for reliability improvements in a manufacturing process by preventing defects due to delamination, cracks, and the like.

According to an aspect of the present inventive concept, an inductor includes: a magnetic body including a magnetic substance; a substrate disposed within the magnetic body; and an internal electrode disposed on at least one of an upper surface and a lower surface of the substrate, the substrate being disposed on an inclined with respect to at least one surface of the magnetic body.

10 In addition, a minimum distance of the distances from the upper and lower surfaces of the magnetic body to the portion thereof to which the substrate is exposed may be 60  $\mu$ m or more.

15 In addition, when the internal electrode is disposed on the upper surface or the lower surface of the substrate to be exposed to one end surface of the magnetic body, a distance from the upper surface of the magnetic body to a portion of the end surface to which the internal electrode is exposed may be 100  $\mu$ m or more, and a distance from the lower surface of the magnetic body to a portion of the end surface to which the internal electrode is exposed may be 150  $\mu$ m or more.

## BRIEF DESCRIPTION OF THE DRAWINGS

The above and other aspects, features, and advantages of the present inventive concept will be more clearly understood from the following detailed description taken in conjunction with the accompanying drawings, in which:

25 FIG. 1 is a perspective view of an inductor according to an embodiment of the present inventive concept;

30 FIG. 2 is a cross-sectional view of the inductor illustrated in FIG. 1, taken along line A-A';

35 FIG. 3 is a perspective view of an inductor according to another embodiment of the present inventive concept;

40 FIG. 4 is a cross-sectional view of the inductor illustrated in FIG. 3, taken along line B-B'; and

45 FIG. 5 is a perspective view of an inductor according to another embodiment of the present inventive concept.

## DETAILED DESCRIPTION OF EMBODIMENTS

Hereinafter, embodiments of the present inventive concept will be described as follows with reference to the attached drawings.

50 The present inventive concept may, however, be exemplified in many different forms and should not be construed as being limited to the specific embodiments set forth herein. Rather, these embodiments are provided so that this disclosure will be thorough and complete, and will fully convey the scope of the disclosure to those skilled in the art.

55 Throughout the specification, it will be understood that when an element, such as a layer, region or wafer (substrate), is referred to as being "on," "connected to," or "coupled to" another element, it can be directly "on," "connected to," or

60 "coupled to" the other element or other elements intervening therebetween may be present. In contrast, when an element is referred to as being "directly on," "directly connected to," or "directly coupled to" another element, there may be no elements or layers intervening therebetween. Like numerals refer to like elements throughout. As used herein, the term "and/or" includes any and all combinations of one or more of the associated listed items.

65 It will be apparent that though the terms first, second, third, etc. may be used herein to describe various members, components, regions, layers and/or sections, these members, components, regions, layers and/or sections should not be

limited by these terms. These terms are only used to distinguish one member, component, region, layer or section from another region, layer or section. Thus, a first member, component, region, layer or section discussed below could be termed a second member, component, region, layer or section without departing from the teachings of the exemplary embodiments.

Spatially relative terms, such as "above," "upper," "below," and "lower" and the like, may be used herein for ease of description to describe one element's relationship to another element(s) as shown in the figures. It will be understood that the spatially relative terms are intended to encompass different orientations of the device in use or operation in addition to the orientation depicted in the figures. For example, if the device in the figures is turned over, elements described as "upper," or "above" other elements would then be oriented "lower," or "below" the other elements or features. Thus, the term "above" can encompass both the above and below orientations depending on a particular direction of the figures. The device may be otherwise oriented (rotated 90 degrees or at other orientations) and the spatially relative descriptors used herein may be interpreted accordingly.

The terminology used herein is for describing particular embodiments only and is not intended to be limiting of the present inventive concept. As used herein, the singular forms "a," "an," and "the" are intended to include the plural forms as well, unless the context clearly indicates otherwise. It will be further understood that the terms "comprises," and/or "comprising" when used in this specification, specify the presence of stated features, integers, steps, operations, members, elements, and/or groups thereof, but do not preclude the presence or addition of one or more other features, integers, steps, operations, members, elements, and/or groups thereof.

Hereinafter, embodiments of the present inventive concept will be described with reference to schematic views illustrating embodiments of the present inventive concept. In the drawings, for example, due to manufacturing techniques and/or tolerances, modifications of the shape shown may be estimated. Thus, embodiments of the present inventive concept should not be construed as being limited to the particular shapes of regions shown herein, for example, to include a change in shape results in manufacturing. The following embodiments may also be constituted by one or a combination thereof.

The contents of the present inventive concept described below may have a variety of configurations and propose only a configuration herein, but are not limited thereto.

FIG. 1 is a perspective view of an inductor 100 according to an embodiment of the present inventive concept. FIG. 2 is a cross-sectional view of the inductor 100 illustrated in FIG. 1, taken along line A-A'.

As shown in FIGS. 1 and 2, a thickness direction of a magnetic body 10 is referred to as "T", a length direction thereof is referred to as "L", and a width direction thereof is referred to as "W". Surfaces facing an upper surface and a lower surface of a substrate 30 disposed inside a magnetic body 10 are defined as an upper surface and a lower surface of the magnetic body 10, respectively. Surfaces through which the substrate 30 is exposed outwardly from the magnetic body 10 are defined as first and second end surfaces of the magnetic body 10, and surfaces adjacent to the first and second end surfaces in the length or width direction are defined as third and fourth side surfaces. In this

case, the upper surface and the lower surface of the magnetic body 10 are adjacent to the first and second end surfaces in the thickness direction.

Referring to FIGS. 1 and 2, the inductor 100 according to an exemplary embodiment of the present inventive concept may include the magnetic body 10 including a magnetic substance, the substrate 30 disposed within the magnetic body 10, and internal electrodes 41 and 42 disposed on at least one of the upper surface and the lower surface of the substrate 30, the substrate 30 being disposed on an incline with respect to at least one surface of the magnetic body 10.

In general, an inductor-manufacturing process may be subjected to a process of cutting a magnetic body (hereinafter referred to as a "bulk magnetic body") for manufacturing a plurality of inductors into individual inductor units. In this case, defects such as cracks, delamination, and the like may occur in the magnetic body mainly from cut surfaces of the magnetic body, due to differences in physical properties among the internal electrodes, the substrate, and the magnetic substance.

In particular, when distances from the upper surface and the lower surface of the magnetic body to the internal electrodes and the substrate are insufficiently secured in order to miniaturize the inductor, the possibility of incurring defects among the internal electrodes, the substrate, and the magnetic body due to stress resulting from the cutting process applied to the magnetic body may be increased.

When distances from the upper surface and the lower surface of the magnetic body to the internal electrodes and the substrate are increased in order to prevent defects such as cracks, delamination, and the like, miniaturization of the inductor may not be feasible. When an area occupied by the internal electrodes is reduced, the capacity of the inductor may be decreased.

In the inductor 100 according to an exemplary embodiment of the present inventive concept, the substrate 30 on which the internal electrodes 41 and 42 are disposed may be disposed on an incline, and thus a size of the magnetic body 10 may be maintained, and distances between the internal electrodes 41 and 42 and the upper surface and the lower surface of the magnetic body 10 may be increased, thereby preventing the occurrence of cracks, delamination, and the like during a cutting process.

In addition, a length of the substrate 30 disposed within the magnetic body 10 may be increased, and thus the area occupied by the internal electrodes 41 and 42 may be increased, thereby increasing the capacity of the inductor 100.

Referring to FIGS. 1 and 2, the substrate 30 disposed within the magnetic body 10 may be exposed to at least one external surface of the magnetic body 10. On the surface of the magnetic body 10 to which the substrate 30 is exposed, a distance from the upper surface of the magnetic body 10 to a portion thereof to which the substrate 30 is exposed may be different from a distance from the lower surface of the magnetic body 10 to the portion thereof to which the substrate 30 is exposed.

In this case, it may be advantageous to dispose the substrate away from the upper surface and the lower surface of the magnetic body in order to prevent cracks from occurring in the vicinity of the substrate positioned on a cut surface of the magnetic body due to stress caused when the bulk magnetic body is cut into respective units. In an exemplary embodiment of the present inventive concept, a minimum distance of the distances from the upper and lower

surfaces of the magnetic body 10 to the portion thereof to which the substrate 30 is exposed may be set to 60  $\mu\text{m}$  or more.

In particular, in the case of the inductor 100 in which a thickness thereof, that is, a distance from the upper surface to the lower surface of the magnetic body 10, is 0.8 mm or less, a minimum distance of the distances from the upper and lower surfaces of the magnetic body 10 to the portion thereof to which the substrate 30 is exposed may preferably be set to 60  $\mu\text{m}$  or more, in order to prevent defects during a cutting process.

In addition, when the substrate 30 is exposed to the first end surface and the second end surface of the magnetic body 10, a distance from the lower surface of the magnetic body 10 to a portion of the first end surface to which the substrate 30 is exposed may be different from a distance from the lower surface of the magnetic body 10 to a portion of the second end surface to which the substrate 30 is exposed. In this case, a minimum distance of the distances from the upper and lower surfaces of the magnetic body 10 to the portions thereof to which the substrate 30 is exposed may be set to 60  $\mu\text{m}$  or more.

Referring to FIGS. 1 and 2, the internal electrode 41 or 42 formed within the magnetic body 10 may be disposed on the upper surface or the lower surface of the substrate 30 to be exposed to one end surface of the magnetic body 10. When the internal electrode 41 or 42 is disposed on the upper surface of the substrate 30 to be exposed to one end surface of the magnetic body 10, a distance from the upper surface of the magnetic body 10 to a portion of the end surface to which the internal electrode 41 or 42 is exposed may preferably be set to 100  $\mu\text{m}$  or more. When the internal electrode 41 or 42 is disposed on the lower surface of the substrate 30 to be exposed to one end surface of the magnetic body 10, a distance from the lower surface of the magnetic body 10 to a portion of the end surface to which the internal electrode 41 or 42 is exposed may preferably be set to 150  $\mu\text{m}$  or more.

Cutting stress occurring when a bulk magnetic body is cut into individual inductor units due to differences in physical properties among the internal electrodes, the substrate, and the magnetic substance filling the magnetic body 10 may more significantly act on spaces between the internal electrodes and the magnetic body, rather than on spaces between the substrate 30 and the magnetic substance. Therefore, distances from the upper and lower surfaces of the magnetic body 10 to the internal electrodes 41 and 42 may preferably be greater than distances from the upper and lower surfaces of the magnetic body 10 to the substrate 30.

As described above, a distance from the upper surface of the magnetic body 10 to a portion of the end surface to which the internal electrode 41 is exposed may preferably be set to 100  $\mu\text{m}$  or more, and a distance from the lower surface of the magnetic body 10 to a portion of the end surface to which the internal electrode 42 is exposed may preferably be set to 150  $\mu\text{m}$  or more. In particular, in the case of the inductor 100 in which a thickness thereof, that is, a distance from the upper surface to the lower surface of the magnetic body 10, is 0.8 mm or less, a distance from the upper surface of the magnetic body 10 to a portion of the end surface to which the internal electrode 41 is exposed may preferably be set to 100  $\mu\text{m}$  or more, and a distance from the lower surface of the magnetic body 10 to a portion of the end surface to which the internal electrode 42 is exposed may preferably be set to 150  $\mu\text{m}$  or more, in order to prevent defects during a cutting process.

In addition, the substrate 30 may be exposed to the first end surface and the second end surface of the magnetic body 10, and the internal electrodes 41 and 42 may include a first internal electrode 41 exposed to the first end surface of the magnetic body 10 and a second internal electrode 42 exposed to the second end surface of the magnetic body 10. When each of the first and second internal electrodes 41 and 42 is disposed on the upper surface or the lower surface of the substrate 30 to be exposed, distances between the first and second internal electrodes 41 and 42 and the upper and lower surfaces of the magnetic body 10 may be set as below.

When the first internal electrode 41 is disposed on the upper surface of the substrate 30 to be exposed to the first end surface of the magnetic body 10, a distance from the upper surface of the magnetic body 10 to a portion of the end surface to which the first internal electrode 41 is exposed may be set to 100  $\mu\text{m}$  or more. When the first internal electrode 41 is disposed on the lower surface of the substrate 30 to be exposed to the first end surface of the magnetic body 10, a distance from the lower surface of the magnetic body 10 to a portion of the end surface to which the first internal electrode 41 is exposed may be set to 150  $\mu\text{m}$  or more. When the second internal electrode 42 is disposed on the upper surface of the substrate 30 to be exposed to the second end surface of the magnetic body 10, a distance from the upper surface of the magnetic body 10 to a portion of the end surface to which the second internal electrode 42 is exposed may be set to 100  $\mu\text{m}$  or more. When the second internal electrode 42 is disposed on the lower surface of the substrate 30 to be exposed to the second end surface of the magnetic body 10, a distance from the lower surface of the magnetic body 10 to a portion of the end surface to which the second internal electrode 42 is exposed may be set to 150  $\mu\text{m}$  or more.

That is, the internal electrode 41 or 42 is exposed outwardly from the magnetic body 110 while being disposed on the upper surface or the lower surface of the substrate 30. When the internal electrode 41 is disposed on the upper surface of the substrate 30 to be exposed outwardly from the magnetic body 110, the internal electrode 41 may be spaced apart from the upper surface of the magnetic body 110 by 100  $\mu\text{m}$  or more. When the internal electrode 42 is disposed on the lower surface of the substrate 30 to be exposed outwardly from the magnetic body 110, the internal electrode 42 may be spaced apart from the lower surface of the magnetic body 110 by 150  $\mu\text{m}$  or more.

Hereinafter, on the basis of FIG. 2, the inductor 100 according to the exemplary embodiment of the present inventive concept will be described in detail.

In FIG. 2, the substrate 30 may be exposed to the first end surface and the second end surface of the magnetic body 10, and a distance A from the lower surface of the magnetic body 10 to a portion of the second end surface thereof to which the substrate 30 is exposed may be shorter than a distance E from the lower surface of the magnetic body 10 to a portion of the first end surface thereof to which the substrate 30 is exposed.

In addition, a distance B from the upper surface of the magnetic body 10 to a portion of the second end surface thereof to which the substrate 30 is exposed may be greater than a distance D from the upper surface of the magnetic body 10 to a portion of the first end surface thereof to which the substrate 30 is exposed.

The internal electrodes 41 and 42 may include the first internal electrode 41 disposed on the upper surface of the substrate 30 to be exposed to the second end surface of the magnetic body 10 and the second internal electrode 42

disposed on the lower surface of the substrate to be exposed to the first end surface of the magnetic body 10.

In this case, the distance A from the lower surface of the magnetic body 10 to a portion of the second end surface thereof to which the substrate 30 is exposed, and the distance D from the upper surface of the magnetic body 10 to a portion of the first end surface thereof to which the substrate 30 is exposed, may be respectively set to 60  $\mu\text{m}$  or more.

In addition, a distance C from the upper surface of the magnetic body 10 to a portion of the second end surface thereof to which the first internal electrode 41 is exposed may be set to 100  $\mu\text{m}$  or more, and a distance F from the lower surface of the magnetic body 10 to a portion of the first end surface thereof to which the second internal electrode 42 is exposed may be respectively set to 150  $\mu\text{m}$  or more.

Through such a configuration, defects during a cutting process may be prevented, and high capacity may be formed as described above.

FIG. 3 is a perspective view of an inductor 200 according to another embodiment of the present inventive concept, and FIG. 4 is a cross-sectional view of the inductor 200 illustrated in FIG. 3, taken along line B-B'.

Referring to FIGS. 3 and 4, the magnetic body 10 may further include an upper cover layer 11 and a lower cover layer 12 disposed, respectively, above and below the substrate 30 and the internal electrodes 41 and 42. The upper cover layer 11 and the lower cover layer 12 may serve to prevent degradation in electrical characteristics of the first and second internal electrodes 41 and 42.

In FIGS. 3 and 4, the substrate 30 may be exposed to the first and second end surfaces of the magnetic body 10, and a distance L from the lower surface of the magnetic body 10 to a portion of the first end surface thereof to which the substrate 30 is exposed may be shorter than a distance P from the lower surface of the magnetic body 10 to a portion of the second end surface thereof to which the substrate 30 is exposed.

In addition, a distance M from the upper surface of the magnetic body 10 to a portion of the first end surface thereof to which the substrate 30 is exposed may be greater than a distance O from the upper surface of the magnetic body 10 to a portion of the second end surface thereof to which the substrate 30 is exposed.

The internal electrodes 41 and 42 may include the first internal electrode 41 disposed on the upper surface of the substrate 30 to be exposed to the first end surface of the magnetic body 10 and the second internal electrode 42 disposed on the lower surface of the substrate 30 to be exposed to the second end surface of the magnetic body 10.

In this case, the distance L from the lower surface of the magnetic body 10 to a portion of the first end surface thereof to which the substrate 30 is exposed and the distance O from the upper surface of the magnetic body 10 to a portion of the second end surface thereof to which the substrate 30 is exposed may be respectively set to 60  $\mu\text{m}$  or more.

In addition, a distance N from the upper surface of the magnetic body 10 to a portion of the first end surface thereof to which the first internal electrode 41 is exposed may be set to 100  $\mu\text{m}$  or more, and a distance Q from the lower surface of the magnetic body 10 to a portion of the second end surface thereof to which the second internal electrode 42 is exposed may be set to 150  $\mu\text{m}$  or more.

FIG. 5 is a perspective view of an inductor 300 according to another embodiment of the present inventive concept.

Referring to FIG. 5, an inductor 300 according to an exemplary embodiment of the present inventive concept may further include first and second external electrodes 81

and 82 disposed on the first and second end surfaces of the magnetic body 10 to be connected to the first and second internal electrodes 41 and 42, respectively.

Hereinafter, respective components configuring the inductor 100 according to the exemplary embodiment of the present inventive concept will be described.

A material of the magnetic body 10 is not limited, as long as the material may form the exterior of the inductor 100 and exhibit magnetic properties. For example, the magnetic body 10 may be formed by providing a ferrite material or magnetic metal powder.

The ferrite material maybe a ferrite material commonly known in the art such as an Mn—Zn based ferrite, an Ni—Zn based ferrite, an Ni—Zn—Cu based ferrite, an Mn—Mg based ferrite, a Ba based ferrite, an Li based ferrite, or the like.

The magnetic metal powder may contain at least one selected from the group consisting of Fe, Si, Cr, Al, and Ni. For example, the magnetic metal powder may contain Fe—Si—B—Cr based amorphous metal particles, but is not limited thereto.

The magnetic metal powder may have a particle diameter of 0.1  $\mu\text{m}$  to 30  $\mu\text{m}$  and may be included in a form in which magnetic metal powder particles are dispersed in a thermoplastic resin such as an epoxy resin, polyimide, or the like.

The internal electrodes 41 and 42 disposed within the magnetic body 10 may be formed as spiral shaped coils.

The first internal electrode 41 having a coil shape may be formed on a first surface of the substrate 30 disposed within the magnetic body 10, and the second internal electrode 42 having a coil shape may be formed on a second surface opposing the first surface of the substrate 30. The first and second internal electrodes 41 and 42 may be electrically connected to each other through vias (not shown) formed in the substrate 30.

The first and second internal electrodes 41 and 42 may be formed by an electroplating method.

The internal electrodes and vias (not shown) may contain a metal having excellent electrical conductivity, such as silver (Ag), palladium (Pd), aluminum (Al), nickel (Ni), titanium (Ti), gold (Au), copper (Cu), platinum (Pt), or alloys thereof.

The internal electrodes 41 and 42 may be coated with an insulating layer 50. The insulating layer 50 may be formed by an exposure or development process such as screen printing or photoresist (PR), or a spray coating process, commonly known in the art.

The insulating layer 50 may contain one or more materials selected from the group of epoxy, polyimide, and a liquid crystalline polymer (LCP), but is not limited thereto. The internal electrodes 41 and 42 may be coated with the insulating layer 50 and may not be in direct contact with a magnetic material forming the magnetic body 10.

The substrate 30 may be formed as, for example, a polypropylene glycol (PPG) substrate, a ferrite substrate, a metallic soft-magnetic material, or the like. A through hole may be formed to penetrate through a central portion of the substrate 30 and may be filled with a magnetic material to form a core part 55. In accordance with the formation of the core part 55 filled with a magnetic material, inductance Ls may be improved.

One end portion of the first internal electrode 41 formed on one surface of the substrate 30 may be exposed to one end surface of the magnetic body 10 in the length direction (L), and one end portion of the second internal electrode 42

formed on the other surface of the substrate 30 may be exposed to the other end surface of the magnetic body 10 in the length direction (L).

The internal electrodes 41 and 42 exposed to the both end surfaces of the magnetic body 10 in the length direction (L) may be connected to the first and second external electrodes 81 and 82 to be electrically connected thereto.

The first and second external electrodes 81 and 82 may contain a metal having excellent electrical conductivity, such as nickel (Ni), copper (Cu), tin (Sn), silver (Ag), or the like, alone or in combination.

### EXAMPLES

Tables 1 and 2 show comparative results obtained by observing process defects in inductors (Inventive Examples) according to an exemplary embodiment of the present inventive concept and in inductors (Comparative Examples) not in compliance with the exemplary embodiment of the present inventive concept, and measuring capacity degrees of the inductors. Table 1 was obtained by observing the occurrence of process defects depending on a distance from an upper surface of a magnetic body to a substrate and a distance from the upper surface of the magnetic body to an internal electrode. Table 2 was obtained by observing the occurrence of process defects depending on a distance from a lower surface of the magnetic body to the substrate and a distance from the lower surface of the magnetic body to an internal electrode.

In Tables 1 and 2, inductors each including a magnetic body having a thickness of 0.6 mm were used in the Inventive Examples and the Comparative Examples. In the examples of Table 1, a distance from the lower surface of the magnetic body to the internal electrode exposed to one end surface of the magnetic body was set to 150 µm or more. In the examples of Table 2, a distance from the upper surface of the magnetic body to the internal electrode exposed to one end surface of the magnetic body was set to 100 µm or more.

In Tables 1 and 2, the Inventive Examples were manufactured in such a manner that the substrate thereof was inclined, and distances from the upper and lower surfaces of the magnetic body to the substrate exposed to end surfaces of the magnetic body were set to 60 µm or more.

In Table 1, Comparative Example 1 was manufactured by not inclining the substrate, while Comparative Examples 2 to 9 were manufactured by inclining the substrate. In Table 2, Comparative Example 10 was manufactured by not inclining the substrate, while Comparative Examples 11 to 18 were manufactured by inclining the substrate.

The occurrence of process defects was confirmed by cutting the inductors according to the inventive and comparative examples to observe the occurrence of cracks, delamination, edge tearing, and the like, through scanning electron microscope (SEM) measurement.

TABLE 1

|                       | Inclination of Substrate | Distance from Upper Surface to Substrate (µm) | Distance from Upper Surface to Internal Electrode (µm) | Process Defects |
|-----------------------|--------------------------|-----------------------------------------------|--------------------------------------------------------|-----------------|
| Comparative Example 1 | Absent                   | —                                             | —                                                      | Occurred        |
| Comparative Example 2 | Present                  | 20                                            | 80                                                     | Occurred        |

TABLE 1-continued

|                       | Inclination of Substrate | Distance from Upper Surface to Substrate (µm) | Distance from Upper Surface to Internal Electrode (µm) | Process Defects |
|-----------------------|--------------------------|-----------------------------------------------|--------------------------------------------------------|-----------------|
| Comparative Example 3 | Present                  | 20                                            | 100                                                    | Occurred        |
| Comparative Example 4 | Present                  | 20                                            | 130                                                    | Occurred        |
| Comparative Example 5 | Present                  | 40                                            | 80                                                     | Occurred        |
| Comparative Example 6 | Present                  | 40                                            | 100                                                    | Occurred        |
| Comparative Example 7 | Present                  | 40                                            | 130                                                    | Occurred        |
| Comparative Example 8 | Present                  | 60                                            | 80                                                     | Occurred        |
| Inventive Example 1   | Present                  | 60                                            | 100                                                    | Not Occurred    |
| Inventive Example 2   | Present                  | 80                                            | 130                                                    | Not Occurred    |
| Comparative Example 9 | Present                  | 80                                            | 80                                                     | Occurred        |
| Inventive Example 3   | Present                  | 80                                            | 100                                                    | Not Occurred    |
| Inventive Example 4   | Present                  | 80                                            | 130                                                    | Not Occurred    |

TABLE 2

|                        | Inclination of Substrate | Distance from Lower Surface to Substrate (µm) | Distance from Lower Surface to Internal Electrode (µm) | Process Defects |
|------------------------|--------------------------|-----------------------------------------------|--------------------------------------------------------|-----------------|
| Comparative Example 10 | Absent                   | —                                             | —                                                      | Occurred        |
| Comparative Example 11 | Present                  | 20                                            | 130                                                    | Occurred        |
| Comparative Example 12 | Present                  | 20                                            | 150                                                    | Occurred        |
| Comparative Example 13 | Present                  | 20                                            | 170                                                    | Occurred        |
| Comparative Example 14 | Present                  | 40                                            | 130                                                    | Occurred        |
| Comparative Example 15 | Present                  | 40                                            | 150                                                    | Occurred        |
| Comparative Example 16 | Present                  | 40                                            | 170                                                    | Occurred        |
| Comparative Example 17 | Present                  | 60                                            | 130                                                    | Occurred        |
| Inventive Example 5    | Present                  | 60                                            | 150                                                    | Not Occurred    |
| Inventive Example 6    | Present                  | 80                                            | 170                                                    | Not Occurred    |
| Comparative Example 18 | Present                  | 80                                            | 130                                                    | Occurred        |
| Inventive Example 7    | Present                  | 80                                            | 150                                                    | Not Occurred    |
| Inventive Example 8    | Present                  | 80                                            | 170                                                    | Not Occurred    |

As shown in Table 1, process defects did not occur when the substrate was inclined, the distance from the upper

## 11

surface of the magnetic body to the substrate was 60  $\mu\text{m}$  or more, and the distance from the upper surface of the magnetic body to the internal electrode was 100  $\mu\text{m}$  or more.

As shown in Table 2, process defects did not occur when the substrate was inclined, the distance from the lower surface of the magnetic body to the substrate was 60  $\mu\text{m}$  or more, and the distance from the lower surface of the magnetic body to the internal electrode was 150  $\mu\text{m}$  or more.

As set forth above, according to embodiments of the present inventive concept, an inductor having high capacity characteristics and allowing for reliability improvements in a manufacturing process by preventing defects due to delamination, cracks, and the like, may be provided.

While the present inventive concept has been shown and described in connection with the embodiments, it will be apparent to those skilled in the art that modifications and variations can be made without departing from the spirit and scope of the invention as defined by the appended claims.

What is claimed is:

## 1. An inductor comprising:

a magnetic body including a magnetic substance;  
a substrate disposed within the magnetic body; and  
an internal electrode disposed as a plurality of turns on a

planar surface of the substrate,  
wherein the planar surface of the substrate is disposed on an incline with respect to at least one of opposing upper and lower surfaces of the magnetic body, the planar surface of the substrate is spaced away from the opposing upper and lower surfaces of the magnetic body, and the incline of the planar surface of the substrate is monotonic across a diameter of the plurality of turns.

## 2. The inductor of claim 1, wherein the substrate is exposed to at least one external surface of the magnetic body, and

a distance from the upper surface of the magnetic body to a portion of the at least one external surface to which the substrate is exposed is different from a distance from the lower surface of the magnetic body to the portion of the at least one external surface to which the substrate is exposed.

3. The inductor of claim 2, wherein a minimum distance of the distances from the upper and lower surfaces of the magnetic body to the portion of the at least one external surface to which the substrate is exposed is 60  $\mu\text{m}$  or more.

## 4. The inductor of claim 2, wherein the internal electrode is exposed to an end surface of the magnetic body,

wherein when the internal electrode is disposed on an upper surface of the substrate to be exposed to the end surface of the magnetic body, a distance from the upper surface of the magnetic body to a portion of the end surface to which the internal electrode is exposed is 100  $\mu\text{m}$  or more, and

wherein when the internal electrode is disposed on a lower surface of the substrate to be exposed to the end surface of the magnetic body, a distance from the lower surface of the magnetic body to a portion of the end surface to which the internal electrode is exposed is 150  $\mu\text{m}$  or more.

## 5. The inductor of claim 1, wherein a distance from the upper surface to the lower surface of the magnetic body is 0.8 mm or less.

## 6. The inductor of claim 1, wherein the magnetic body further includes an upper cover layer and a lower cover layer disposed above and below the substrate and the internal electrodes, respectively.

## 12

7. The inductor of claim 1, wherein the internal electrode is exposed to at least one end surface of the magnetic body, and

a minimum distance between an exposed portion of the internal electrode and one surface of the upper and lower surfaces of the magnetic body is longer than a minimum distance between an exposed portion of the substrate and a remaining surface of the upper and lower surfaces of the magnetic body.

## 8. The inductor of claim 1, wherein the substrate is exposed to first and second end surfaces of the magnetic body, and a distance from the lower surface of the magnetic body to a portion of the first end surface at which the substrate is exposed is different from a distance from the lower surface of the magnetic body to a portion of the second end surface at which the substrate is exposed.

## 9. The inductor of claim 1, wherein the planar surface of the substrate having the internal electrode disposed thereon is planar across an entirety of the diameter of the plurality of turns.

## 10. The inductor of claim 1, wherein the planar surface of the substrate disposed on the incline and having the internal electrode disposed thereon has a substantially constant thickness.

## 11. An inductor comprising:

a magnetic body including a magnetic substance;  
a substrate disposed within the magnetic body; and  
an internal electrode disposed on a planar surface of the

substrate,  
wherein the planar surface of the substrate is disposed on an incline with respect to at least one of opposing upper and lower surfaces of the magnetic body and is spaced away from the opposing upper and lower surfaces of the magnetic body,

the substrate is exposed to first and second end surfaces of the magnetic body, and  
a distance from the lower surface of the magnetic body to a portion of the first end surface at which the substrate is exposed is different from a distance from the lower surface of the magnetic body to a portion of the second end surface at which the substrate is exposed.

12. The inductor of claim 11, wherein a minimum distance of the distances from the upper and lower surfaces of the magnetic body to the portions thereof at which the substrate is exposed is 60  $\mu\text{m}$  or more.

## 13. The inductor of claim 11, wherein the internal electrode includes a first internal electrode exposed to the first end surface of the magnetic body and a second internal electrode exposed to the second end surface of the magnetic body, each of the first and second internal electrodes being disposed on an upper surface or a lower surface of the substrate,

wherein when the first internal electrode is disposed on the upper surface of the substrate to be exposed to the first end surface of the magnetic body, a distance from the upper surface of the magnetic body to a portion of the end surface at which the first internal electrode is exposed is 100  $\mu\text{m}$  or more,

wherein when the first internal electrode is disposed on the lower surface of the substrate to be exposed to the first end surface of the magnetic body, a distance from the lower surface of the magnetic body to a portion of the end surface at which the first internal electrode is exposed is 150  $\mu\text{m}$  or more,

wherein when the second internal electrode is disposed on the upper surface of the substrate to be exposed to the second end surface of the magnetic body, a distance

**13**

from the upper surface of the magnetic body to a portion of the end surface at which the second internal electrode is exposed is 100  $\mu\text{m}$  or more, and  
 wherein when the second internal electrode is disposed on the lower surface of the substrate to be exposed to the second end surface of the magnetic body, a distance from the lower surface of the magnetic body to a portion of the end surface at which the second internal electrode is exposed is 150  $\mu\text{m}$  or more.

**14.** The inductor of claim **11**, wherein the distance from the lower surface of the magnetic body to the portion of the first end surface at which the substrate is exposed is shorter than the distance from the lower surface of the magnetic body to the portion of the second end surface at which the substrate is exposed.

**15.** The inductor of claim **14**, wherein the internal electrode includes a first internal electrode disposed on an upper surface of the substrate to be exposed to the first end surface

**14**

of the magnetic body and a second internal electrode disposed on a lower surface of the substrate to be exposed to the second end surface of the magnetic body, and

the distance from the lower surface of the magnetic body to the portion of the first end surface thereof at which the substrate is exposed, and a distance from the upper surface of the magnetic body to the portion of the second end surface thereof at which the substrate is exposed, are respectively 60  $\mu\text{m}$  or more.

**16.** The inductor of claim **14**, wherein a distance from the upper surface of the magnetic body to a portion of the first end surface thereof at which a first internal electrode is exposed, and a distance from the lower surface of the magnetic body to a portion of the second end surface thereof at which a second internal electrode is exposed, are respectively 150  $\mu\text{m}$  or more.

\* \* \* \* \*